

1

3,672,906

**SILVER HALIDE EMULSIONS SENSITIZED WITH  
METHINE DYES CONTAINING A CYCLO-  
PENTANONE NUCLEUS**

Leslie G. S. Brooker, Rochester, and Arthur Fumia, Jr.,  
Hilton, N.Y., assignors to Eastman Kodak Company,  
Rochester, N.Y.

No Drawing. Continuation-in-part of application Ser. No.  
656,647, July 28, 1967. This application Mar. 25, 1970,  
Ser. No. 22,707

Int. Cl. G03c 1/08

U.S. Cl. 96—142

8 Claims

**ABSTRACT OF THE DISCLOSURE**

Novel methine dyes containing a cyclopentanone nucleus in the methine chain are prepared by the acid hydrolysis of cyanine enamine derivatives. These methine dyes are spectral sensitizers for photographic silver halide emulsions. A number of the new dyes extend the sensitivity of photographic silver halide emulsions into the red and near infra-red regions of the spectrum.

2

spectrally sensitized with a methine dye comprising a nitrogen-containing heterocyclic nucleus having from 5 to 6 atoms in the heterocyclic ring, said nucleus being of the type used in cyanine dyes, said heterocyclic nucleus being joined by a dimethine linkage to the 2-carbon atom of a cyclopentanone nucleus.

Especially useful dyes which sensitize photographic silver halide emulsions to infra-red radiation are those which comprise first and second nitrogen-containing heterocyclic nuclei containing from 5 to 6 atoms in the heterocyclic ring, said nuclei being of the type used in cyanine dyes, said first nucleus being joined by a dimethine linkage to the 2-carbon atom of a cyclopentanone ring, and said second nucleus being joined by a dimethine linkage to the 5-carbon atom of said cyclopentanone nucleus.

The preferred cyanine dyes of the invention are represented by the following general formulas:

I.



and

II.



This application is a continuation-in-part of our co-pending U.S. application Ser. No. 656,647 filed July 28, 1967, now abandoned.

This invention relates to novel photographic materials, and more particularly to photographic silver halide emulsions spectrally sensitized with methine dyes.

We have now found that certain methine dyes are excellent spectral sensitizers for both black and white and color photographic silver halide materials. A number of these new dyes extend the sensitivity of photographic silver halide emulsions into the red and near infra-red regions of the spectrum.

It is one object of this invention to provide light sensitive silver halide spectrally sensitized with methine dyes.

Another object of this invention is to provide photographic silver halide emulsions containing certain methine dyes.

Other objects of this invention will become apparent from a consideration of the general description and examples, and the appended claims.

In accordance with one embodiment of this invention, light sensitive photographic silver halide emulsions are

wherein *m* and *n* each represents a positive integer of from 1 to 2, and R and R<sub>1</sub> each represents an alkyl group, preferably a lower alkyl containing from 1 to 4 carbon atoms, e.g., methyl, ethyl, propyl, isopropyl, butyl, hexyl, decyl, dodecyl, etc., a substituted alkyl group, preferably a lower group containing 1 to 4 carbon atoms, such as a hydroxyalkyl group, e.g.,  $\beta$ -hydroxyethyl,  $\gamma$ -hydroxypropyl,  $\omega$ -hydroxybutyl, etc., an alkoxyalkyl group, e.g.,  $\beta$ -methoxyethyl,  $\omega$ -butoxybutyl, etc., a carboxyalkyl group, e.g.,  $\beta$ -carboxyethyl,  $\omega$ -carboxybutyl, etc., a sulfoalkyl group, e.g.,  $\beta$ -sulfoethyl,  $\omega$ -sulfobutyl, etc., a sulfatoalkyl group, e.g.,  $\beta$ -sulfatoethyl,  $\omega$ -sulfatobutyl, etc., an acyloxyalkyl group, e.g.,  $\beta$ -acetoxyethyl,  $\omega$ -propionyloxybutyl, etc., an alkoxy carbonylalkyl group, e.g.,  $\beta$ -methoxycarbonylethyl,  $\omega$ -ethoxycarbonylbutyl, etc., or an aralkyl group, e.g., benzyl, phenethyl, etc., an alkenyl group such as allyl or 1-propenyl, or, an aryl group, e.g., phenyl, naphthyl, tolyl, chlorophenyl, sulfo-phenyl, carboxyphenyl, etc.; and, Z and Z<sub>1</sub> each represents the nonmetallic atoms required to complete a 5- to

6-membered heterocyclic nucleus such as a thiazole nucleus (e.g., thiazole, methylthiazole, 4-phenylthiazole, 5-

## 3

methylthiazole, 5-phenylthiazole, 4,5-dimethylthiazole, 4,5-diphenylthiazole, 4-(2-thienyl)thiazole, etc.), a benzothiazole nucleus (e.g., benzothiazole, 4-chlorobenzothiazole, 5-chlorobenzothiazole, 6-chlorobenzothiazole, 7-chlorobenzothiazole, 4-methylbenzothiazole, 4-methylbenzothiazole, 6-methylbenzothiazole, 5-bromobenzothiazole, 6-bromobenzothiazole, 4-phenylbenzothiazole, 5-phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole, tetrahydrobenzothiazole, 5,6-dimethoxybenzothiazole, 5,6-dioxymethylenebenzothiazole, 5-hydroxybenzothiazole, 6-hydroxybenzothiazole, etc.), an oxazole nucleus (e.g., 4-methyloxazole, 5-methyloxazole, 4-phenyloxazole, diphenyloxazole, 4-ethyloxazole, 4,5-dimethylloxazole, 5-phenyloxazole, etc.), a benzoxazole nucleus (e.g., benzoxazole, 5-chlorobenzoxazole, 5-methylbenzoxazole, 5-phenylbenzoxazole, 6-methylbenzoxazole, 5,6-dimethylbenzoxazole, 4,6-dimethylbenzoxazole, 5-methoxybenzoxazole, 5-ethoxybenzoxazole, 6-chlorobenzoxazole, 6-methoxybenzoxazole, 5-hydroxybenzoxazole, 6-hydroxybenzoxazole, etc.), a naphthoxazole nucleus (e.g.,  $\alpha$ -naphthoxazole,  $\beta,\beta$ -naphthoxazole,  $\beta$ -naphthoxazole, etc.), those of the selenazole series (e.g., 4-methylselenazole, 4-phenylselenazole, etc.), a benzoselenazole nucleus

Formula I above can be readily prepared by hydrolysis of a compound of the general formula:

III.



5

wherein  $n$ , R and Z are as previously defined, and X represents an acid anion such as chloride, bromide, iodide, thiocyanate, sulfamate, perchlorate, p-toluenesulfonate, methyl sulfate, ethyl sulfate, etc., in an aqueous solution of a strong mineral acid such as hydrochloric acid, sulfuric acid, etc., at elevated temperatures and preferably at refluxing temperatures of the reaction mixture, until the hydrolysis reaction is completed. The dye products are then separated from the reaction mixtures by chilling and purified by one or more recrystallizations from suitable solvents such as pyridine methanol etc.

The new cyanine dyes of the invention as defined by Formula II above are prepared by a similar hydrolysis method as described above, except that here the compound that is hydrolyzed is represented by the following general formula:



wherein  $m$ ,  $n$ , R,  $R_1$ , X, Z and  $Z_1$  are as previously defined.

The intermediate dye compounds defined by Formula III above can be conveniently prepared by condensing approximately 1 mole of N-cyclopentenylpyrrolidine with 1 mole of a compound of the general formula:

50 V.



wherein  $n$ , R, X and Z are as previously defined.

The symmetrical intermediate dye compounds defined by Formula IV above can be conveniently prepared for example, by condensing approximately 1 mole N-cyclopentenylpyrrolidine with 2 moles of a compound selected from above Formula V. To prepare the unsymmetrical intermediate dye compounds of Formula IV above, an appropriate compound of Formula III above is condensed with an appropriate compound of Formula V above, in approximately equimolar proportions.

For further details concerning the preparation of cyanine dye intermediates defined by Formulas III and IV above, reference can be had to copending application of R. A. Jeffreys, Ser. No. 518,010, filed Jan. 3, 1966, wherein the preparation of such intermediate dyes are described and claimed.

The following examples further illustrate this invention.

(e.g., benzoselenazole, 5-chloroselenazole, 5-methoxybenzoselenazole, 5-hydroxybenzoselenazole, tetrahydrobenzoselenazole, etc.), a naphthoselenazole nucleus (e.g.,  $\alpha$ -naphthoselenazole,  $\beta,\beta$ -naphthoselenazole,  $\beta$ -naphthoselenazole, etc.), a thiazoline nucleus (e.g., thiazoline, 4-methylthiazoline, etc.), a 2-quinoline nucleus (e.g., quinoline, 3-methylquinoline, 5-methylquinoline, 7-methylquinoline, 8-methylquinoline, 6-chloroquinoline, 6-methoxyquinoline, 6-ethoxyquinoline, 6-hydroxyquinoline, 8-hydroxyquinoline, etc.), a 4-quinoline nucleus (e.g., 6-methoxy-4-quinoline, 7-methyl-4-quinoline, etc.), a 1-isoquinoline nucleus (e.g., 1-isoquinoline, 3,4-dihydro-1-isoquinoline, etc.), a 3-isoquinoline nucleus (e.g., 3-isoquinoline, etc.), a 3,3-dialkylindolenine nucleus (e.g., 3,3-dimethylindolenine, 3,3,5-trimethylindolenine, 3,3,7-trimethylindolenine, etc.), a 2-pyridine nucleus (e.g., pyridine, 3-methylpyridine, 4-methylpyridine, 5-methylpyridine, 3,4-dimethylpyridine, 4-chloropyridine, 3-hydroxypyridine, 3-phenylpyridine, etc.), a 4-pyridine nucleus (e.g., 2-methylpyridine, 3-methylpyridine, 3-chloropyridine, 2,6-dimethylpyridine, 3-hydroxypyridine, etc., a 1-alkylimidazole nucleus (e.g., 1-methylimidazole, 1-ethyl-4-phenylimidazole, 1-butyl-4,5-dimethylimidazole, etc.), a 1-alkylbenzimidazole nucleus (e.g., 1-methylbenzimidazole, 1-butyl-4-methylbenzimidazole, 1-ethyl-5,6-dichlorobenzimidazole, etc.), a 1-alkylnaphthimidazole nucleus (e.g., 1-ethyl- $\alpha$ -naphthimidazole, 1-methyl- $\beta$ -naphthimidazole, etc.), and the like. The symmetrical dyes of the invention coming under Formula II above which contain benzothiazole nuclei are particularly useful spectral sensitizers for photographic silver halide emulsions and are preferred.

The new cyanine dyes of the invention as defined by

75

5  
EXAMPLE 1

2,5-bis[(3-ethyl-2-benzothiazolinylidene)ethylidene]cyclopentanone



3,3'-diethyl - 10,12 - ethylene - 11 - (1-pyrrolidinyl)thiatricarbocyanine iodide (6.4 g., 1 mol.), water (25 ml.), and 36% hydrochloric acid (2 ml.) are mixed and heated under reflux with stirring. The mixture was diluted several times with additional acid and water, with refluxing, continued until the absorption of the starting material had disappeared. After chilling, the solid is collected on a funnel, washed with acetone and dried. After two recrystallizations from pyridine/methanol, the yield of purified dye is 2.1 g. (46%). M.P. 246-247° C. decomposes.

In place of the 3,3'-diethyl-10,12-ethylene-11-(1-pyrrolidinyl) thiacarbocyanine iodide in the above example, there can be substituted an equivalent amount of, for example, 3,3' - diethyl-10,12-ethylene-11-(1-pyrrolidinyl) oxatricarbocyanine salt such as the chloride, bromide, iodide, etc. or a 3,3'-diethyl-10,12-ethylene-11-(1-pyrrolidinyl) selenotriacarbocyanine salt or a 3,3'-diethyl-10,12-ethylene - 11-(1-pyrrolidinyl)thiazotriacarbocyanine salt, and the like, to give the corresponding cyanine dyes of the invention having generally similar spectral sensitizing properties when incorporated in photographic silver halide emulsions.

## EXAMPLE 2

2,5-bis[(1-ethylnaphtho[1,2-d]thiazolin-2-ylidene)ethylidene]cyclopentanone



3,3'-diethyl - 10,12 - ethylene-11-(1-pyrrolidinyl)-4,5,4',5'-dibenzothiacarbocyanine p-toluenesulfonate (3.9 g., 1 mol.), water (75 ml.) ethanol (200 ml.) and 36% hydrochloric acid (5 ml.) are heated under reflux with stirring. The mixture is diluted several times with additional acid and water with refluxing continued until the absorption of the starting material has disappeared. After chilling, the solid is collected on a funnel, washed with methanol and dried. After two recrystallizations from pyridine/methanol, the yield of purified dye is 0.9 g. (32%). M.P. 275-276° C. dec.

In place of the 3,3'-diethyl-10,12-ethylene-(1-pyrrolidinyl) - 4,5,4',5' - dibenzothiacarbocyanine p-toluenesulfonate in the above example there can be substituted an equivalent amount of, for example, 3,3'-diethyl-10,12-ethylene-(1-pyrrolidinyl) - 4,5,4',5' - dibenzoxacarbocyanine salt such as the chloride, bromide iodide, etc., to give the corresponding cyanine dye of the invention having generally similar spectral sensitizing properties for photographic silver halide emulsions.

6  
EXAMPLE 3

2,5-bis[(1,3,3-trimethyl-2-indolinylidene)ethylidene]cyclopentanone



10,12-ethylene - 1,1',3,3,3',3' - hexamethyl-11-(1-pyrrolidinyl)indotriacarbocyanine iodide (6.3 g. 1 mol.) is treated with water and 36% hydrochloric acid in the same manner as Example 2. After two recrystallizations from pyridine/methanol the yield of purified dye is 1.1 g. (25%). M.P. 265-266° C. dec.

## EXAMPLE 4

2-[(3-ethyl-2-benzothiazolinylidene)ethylidene]cyclopentanone



3 - ethyl-2-[2-[2-(1-pyrrolidinyl)cyclopentenyl]vinyl]benzothiazolium iodide (6.0 g. 1 mol.) is treated with water and 36% hydrochloric acid in the manner as Example 2. After two recrystallization from pyridine/methanol, the yield of purified dye is 1.1 g. (31%), M.P. 230-231° C. dec.

In place of the 3-ethyl-2-[2-[2-(1-pyrrolidinyl)cyclopentenyl]vinyl]benzothiazolium iodide in the above example, there can be substituted an equivalent amount of, for example, 3-ethyl-2-[2-[2-(1-pyrrolidinyl)cyclopentenyl]vinyl]benzoxazolium salt such as the bromide, chloride, iodide, etc., or the corresponding selenazolium salts, or the corresponding thiazolium salts, and the like, to give the corresponding cyanine dyes of the invention that likewise extend the sensitivity of photographic silver halide emulsions.

The above prepared dyes of the invention are then tested in a silver chlorobromide emulsion. The dyes, dissolved in suitable solvents, is added to separate portions of the emulsion, at the concentrations indicated in the following Table 1. The dyes are exposed to a minimum amount of radiation after preparation and during addition to the emulsion. When illumination is necessary in handling the dyes, a safelight of the type used in coating panchromatic sensitized silver halide emulsions is employed. After digestion at 50-52° C. for about 10 minutes, the emulsions are coated at a coverage of 459 mg. of silver and 1040 mg. of gelatin per square foot on a cellulose acetate film support. A sample of each coating is exposed on an Eastman 1B sensitometer and to a wedge spectrograph, processed for 5 minutes in Kodak DK-50 developer ("Handbook of Chemistry and Physics," 30th edition, 1947, Chemical Rubber Publishing Co., Cleveland, Ohio, page 2558) having the following composition:

|                                | G.   |
|--------------------------------|------|
| N-methyl-p-aminophenol sulfate | 2.5  |
| Sodium sulfite (desiccated)    | 30.0 |
| Hydroquinone                   | 2.5  |
| Sodium metaborate              | 10.0 |
| Potassium bromide              | 0.5  |
| Water to make 1.0 liter.       |      |

and then fixed in a conventional sodium thiosulfate fixing bath, washed and dried. The sensitizing values obtained are shown in the following Table 1.

TABLE 1

| Dye of Example No. | Dye and concentration (g./mole silver) | Emulsion type        | Sensitization (m $\mu$ ) |
|--------------------|----------------------------------------|----------------------|--------------------------|
|                    |                                        | Range                | Maximum                  |
| 1                  | 0.103                                  | Silver chlorobromide | 760 to 810 (1)           |
| 2                  | 0.13                                   | do                   | 500 to 705               |
| 3                  | 0.102                                  | do                   | 540 to 780               |
| 4                  | 0.13                                   | do                   | To 550                   |
|                    |                                        |                      | 515                      |

<sup>1</sup> No definite maximum.

The following examples illustrate the preparation of the intermediate dye compounds employed in the procedures of above Examples 1 to 4 to prepare the cyanine dyes of the invention. As indicated previously, additional details for the preparation of these and related dye intermediates can be had by reference to the aforementioned R. A. Jeffreys copending application, Ser. No. 518,010, filed Jan. 3, 1966.

## EXAMPLE 5

## 3,3'-diethyl-10,12-ethylene-11-(1-pyrrolidinyl) triatricarbocyanine iodide



N-cyclopentenylpyrrolidine (0.7 gram), 2-[2-acetanilidovinyl] - 3 - ethylbenzothiazolium iodide (4.5 grams) and sodium acetate (0.8 gram) in acetic anhydride (25 ml.) are refluxed together for  $\frac{1}{4}$  hour, and the resulting blue solution is chilled to precipitate the dye product formed. The dye product is filtered off, washed with ethanol and water, and recrystallized from methanol as moss green needles, M.P. above 345° C., in 1 gram (31%) yield.

## EXAMPLE 6

## 3,3'-diethyl-10,12-ethylene-11-(1-pyrrolidinyl)-4,5,4',5'-dibenzothiatriacarbocyanine p-toluenesulfonate



2 - (2 - anilinovinyl) - 1 - ethyl-naphtho[1,2-d]thiazolium p-toluenesulfonate (21 g., 2 mols. +5%), N-cyclopentenylpyrrolidine (2.7 g., 1 mol.), triethylenediamine (7.4 g., 2 mols. +10%), and acetic anhydride (3.7 ml., 2 mols.) are dissolved in N,N-dimethylacetamide (40 ml.) and heated on a steam bath, with stirring, for one-half hour. After chilling, the crude product is collected on a filter, washed with methanol and dried. After two recrystallizations from methanol, the yield of purified dye is 6.1 g. (39%), M.P. 253-254° C. dec.

5  
10  
15

20  
25

30

35

40

45

50

55

60

65

70

75

## EXAMPLE 7

## 10,12-ethylene-1,1',3,3',3'-hexamethyl-11-(1-pyrrolidinyl)indotriacarbocyanine iodide



10,12-ethylene-1,1',3,3',3'-hexamethyl-11-(1-pyrrolidinyl)indotriacarbocyanine iodide (9.4 g., 2 mols. +5%), N-cyclopentenylpyrrolidine (1.4 g., 1 mol.), and triethylenediamine (2.2 g., 1 mol. +100%) are dissolved in N,N-dimethylacetamide (25 ml.) and heated on a steam bath, with stirring, for 15 minutes. After chilling, the reaction mixture is filtered and the filtrate treated with ether to precipitate the product. The crude product is collected on a filter and after two recrystallizations from methanol, the yield of purified dye is 2.1 g. (33%), M.P. 242-243° C. dec.

## EXAMPLE 8

## 3-ethyl-2-{2-[2-(1-pyrrolidinyl)cyclopentenyl]-vinyl}benzothiazolium iodide



N-cyclopentenylpyrrolidine (2.7 grams) and 2-[2-acetanilidovinyl] - 3 - ethylbenzothiazolium iodide (9 grams) in ethanol (25 ml.) are shaken together at room temperature for  $\frac{1}{2}$  hour. The dye product formed is filtered off and recrystallized from ethanol to remove magenta and blue impurities. The orange dye is obtained as maroon leaflets, M.P. 297-299° C. with decomp. (darkens at 290° C.) in 2.1 grams (23%) yield.

## EXAMPLE 9

## N-cyclopentenylpyrrolidine



This compound is prepared in the manner described by G. Stark, et al., J. Am. Chem. Soc., 85, 216 (1963).

For the preparation of photographic emulsions, the new dyes of the invention are advantageously incorporated in the finished silver halide emulsion and should, of course, be uniformly distributed throughout the emulsion. The method of incorporating dyes in emulsions are relatively simple and well known to those skilled in the art of emulsion making. For example, it is convenient to add the dyes from solutions in appropriate solvents, in which the solvent selected should have no deleterious effect on the ultimate light-sensitive materials. Methanol, isopropanol, pyridine, etc., alone or in combination have proven satisfactory as solvents for the majority of the new dyes of the invention. The type of silver halide emulsions that are sensitized with the new dyes include any of those prepared with hydrophilic colloids that are known to be satisfactory for dispersing light-sensitive

silver halides, for examples, emulsions prepared with hydrophilic colloids, such as natural materials, e.g., gelatin, albumin, agar-agar, gum arabic, alginic acid, etc., and synthetic hydrophilic resins, e.g., polyvinyl alcohol, polyvinyl pyrrolidone, cellulose ethers, partially hydrolyzed cellulose acetate, etc.

The concentration of the new dyes in the emulsions can be widely varied, i.e., generally from about 5 to about 100 mg. per liter of flowable emulsion. The specific concentration will vary according to the type of light-sensitive material in the emulsion and according to the effects desired. The most advantageous dye concentration for any given emulsion can be readily determined by making the tests and observations customarily used in the art of emulsion making. The emulsions are coated to advantage on any of the support materials commonly used for photographic elements, for example, paper, glass, cellulose derivatives, such as cellulose acetate, cellulose acetate-propionate, cellulose nitrate, etc., synthetic resins, such as poly styrene, polyethylene terephthalate and other polyesters, polyamides, such as nylon, and the like.

To prepare a gelatino-silver halide emulsion desensitized with one of the new dyes, the following procedure is satisfactory: A quantity of dye is dissolved in a suitable solvent, and a volume of this solution containing the desired amount of dye is slowly added with intimate mixing to about 1,000 cc. of light-sensitive gelatino-silver halide emulsion. With most of the new dyes, from about 10 to 20 mg. of dye per liter of emulsion suffices to produce the desired sensitizing effect with the ordinary gelatino-silver halides including silver chloride, bromide, bromoiodide, chlorobromide, chlorobromoiodide, etc., emulsions. With fine-grain emulsions which include most of the ordinary employed gelatino-silver chloride emulsions, somewhat larger concentrations of dye may be necessary to secure optimum sensitizing effect. While the preceding has dealt with emulsions comprising gelatin, it will be understood that these remarks apply generally to any emulsions in which a part or all of the gelatin is substituted by another suitable hydrophilic colloid such as those previously mentioned.

The above statements are only illustrative and are not to be understood as limiting the invention in any sense, as it will be apparent that the new dyes can be incorporated by other methods in many of the emulsions customarily used in the art. For instance, in a less preferred method, the dyes can be incorporated by bathing a plate or film bearing an emulsion, in a solution of the dye.

Photographic silver halide emulsions, such as those listed above, containing the sensitizing dyes of the invention can also contain such addenda as chemical sensitizers, e.g., sulfur sensitizers (e.g., allyl thiocarbamide, thiourea, allylisothiocyanate, cystine, etc.), various gold compounds (e.g., potassium chloroaurate, auric trichloride, etc.) (see Baldsiefen U.S. Pat. 2,540,085, issued Feb. 6, 1951; Damschroder U.S. Pat. 2,597,856, issued May 27, 1952 and Yutzy et al. U.S. Pat. 2,597,915, issued May 27, 1952), various palladium compounds such as palladium chloride (Baldsiefen U.S. Pat. 2,540,086, issued Feb. 6, 1951), potassium chloropalladate (Stauffer et al. U.S. Pat. 2,598,079, issued May 27, 1952), etc., or mixtures of such sensitizers; antifoggants, such as ammonium

chloroplatinate (Trivelli et al. U.S. Pat. 2,566,245, issued Aug. 28, 1951), ammonium chloroplatinate (Trivelli et al. U.S. Pat. 2,566,263, issued Aug. 28, 1951), benzotriazole, nitrobenzimidazole, 5-nitroindazole, benzidine, mercaptans, etc. (see Mees—"The Theory of the Photographic Process," MacMillan Pub., 1942, page 460), or mixtures thereof; hardeners, such as formaldehyde (Miller U.S. Pat. 1,763,533, issued June 10, 1930), chrome alum (1,763,533), glyoxal (Brunken U.S. Pat. 1,870,354, issued Aug. 9, 1932), dibromacrolein (Block et al. British Pat. 406,750, accepted Mar. 8, 1934), etc.; color couplers, such as those described in Salminen et al. U.S. Pat. 2,423,730, issued July 7, 1947, Spence and Carroll U.S. Pat. 2,640,776, issued June 2, 1953, etc.; or mixture of such addenda. Dispersing agents for color couplers, such as those set forth in Jolley et al. U.S. Pat. 2,322,027, issued June 15, 1943, and Mannes et al. U.S. Pat. 2,304,940, issued Dec. 15, 1942, can also be employed in the above-described emulsions.

The invention has been described in detail with particular reference to preferred embodiments thereof but it will be understood that variations and modifications can be effected within the spirit and scope of the invention as described hereinabove and as defined in the appended claims.

We claim:

1. A light-sensitive photographic silver halide emulsion spectrally sensitized with a methine dye comprising a heterocyclic nucleus selected from the group consisting of a thiazole nucleus, a benzothiazole nucleus, a naphthothiazole nucleus, a thianaphtheno-7',6',4,5-thiazole nucleus, an oxazole nucleus, a benzoxazole nucleus, a naphthoxazole nucleus, a selenazole nucleus, a benzoselenazole nucleus, a naphthoselenazole nucleus, a 2-quinoline nucleus, a 4-quinoline nucleus, a 1-isoquinoline nucleus, a 3-isoquinoline nucleus, a 3,3-dialkylindolenine nucleus, a pyridine nucleus, an imidazole nucleus, a benzimidazole nucleus and a naphthimidazole nucleus; said heterocyclic nucleus being joined by a dimethine linkage to the 2-carbon atom of a cyclopentanone nucleus.

2. A light-sensitive photographic silver halide emulsion spectrally sensitized with a cyanine dye comprising first and second nitrogen-containing heterocyclic nuclei selected from the group consisting of a thiazole nucleus, a benzothiazole nucleus, an naphthothiazole nucleus, a thianaphtheno-7',6',4,5-thiazole nucleus, an oxazole nucleus, a benzoxazole nucleus, a naphthoxazole nucleus, a selenazole nucleus, a benzoselenazole nucleus, a naphthoselenazole nucleus, a thiazoline nucleus, a 2-quinoline nucleus, a 4-quinoline nucleus, a 1-isoquinoline nucleus, a 3-isoquinoline nucleus, a 3,3-dialkylindolenine nucleus, a pyridine nucleus, an imidazole nucleus, a benzimidazole nucleus and a naphthimidazole nucleus; said first heterocyclic nucleus being joined by a dimethine linkage to the 2-carbon atom of a cyclopentanone nucleus, and said second heterocyclic nucleus being joined by a dimethine linkage to the 5-carbon atom of said cyclopentanone nucleus.

3. A light sensitive photographic silver halide emulsion spectrally sensitized with a methine dye having one of the following formulas:



and



wherein  $m$  and  $n$  each represents a positive integer of from 1 to 2; R and  $R_1$  each represents a member selected from the group consisting of an alkyl group, an allyl group, and an aryl group; and, Z and  $Z_1$  each represents the non-metallic atoms necessary to complete a heterocyclic nucleus selected from the group consisting of a thiazole nucleus, a benzothiazole nucleus, a naphthothiazole nucleus, a thianaphtheno-7',6',4,5-thiazole nucleus, an oxazole nucleus, a benzoxazole nucleus, a naphthoxazole nucleus, a selenazole nucleus, a benzoselenazole nucleus, a naphthoselenazole nucleus, a thiazoline nucleus, a 2-quinoline nucleus, a 4-quinoline nucleus, a 1-isoquinoline nucleus, a 3-isoquinoline nucleus, a 3,3-dialkylindolenine nucleus, a pyridine nucleus, an imidazole nucleus, a benzimidazole nucleus and a naphthimidazole nucleus.

4. A light sensitive photographic silver halide emulsion spectrally sensitized with a methine dye having the following formula:



wherein  $n$  represents a positive integer of from 1 to 2; R represents a member selected from the group consisting of an alkyl group, an allyl group, and an aryl group; and, Z represents the non-metallic atoms necessary to complete a heterocyclic nucleus selected from the group consisting of a thiazole nucleus, a benzothiazole nucleus, a naphthothiazole nucleus, a thianaphtheno-7',6',4,5-thiazole nucleus, an oxazole nucleus, a benzoxazole nucleus, a naphthoxazole nucleus, a selenazole nucleus, an benzoselenazole nucleus, a naphthoselenazole nucleus, a thiazoline nucleus, a 2-quinoline nucleus, a 4-quinoline nucleus, a 1-isoquinoline nucleus, a 3-isoquinoline nucleus, a 3,3-dialkylindolenine nucleus, a pyridine nucleus, an imidazole nucleus, a benzimidazole nucleus and a naphthimidazole nucleus.

5. A light sensitive photographic silver halide emulsion spectrally sensitized with a dye having the following formula:



wherein  $m$  and  $n$  represents a positive integer of from 1 to 2; R and  $R_1$  each represents a member selected from the group consisting of an alkyl group, an allyl group, and an aryl group; and Z and  $Z_1$  each represents the non-metallic atoms necessary to complete a heterocyclic nucleus selected from the group consisting of a thiazole nucleus, a benzothiazole nucleus, a naphthothiazole nucleus, a thianaphtheno-7',6',4,5-thiazole nucleus, an oxazole nucleus, a benzoxazole nucleus, a naphthoxazole nucleus, a selenazole nucleus, a benzoselenazole nucleus, a naphthoselenazole nucleus, a thiazoline nucleus, a 2-quinoline nucleus, a 4-quinoline nucleus, a 1-isoquinoline nucleus, a 3-isoquinoline nucleus, a 3,3-dialkylindolenine nucleus, a pyridine nucleus, an imidazole nucleus, a benzimidazole nucleus and a naphthimidazole nucleus.

20 6. A light sensitive photographic silver halide emulsion spectrally sensitized with a cyanine dye selected from the group consisting of

- 25 2,5-bis[ (3-ethyl-2-benzothiazolinylidene)ethylidene]  
cyclopentanone,  
2,5-bis[ (1-ethylnaphtho[1,2-d]thiazolin-2-ylidene)  
ethylidene]cyclopentanone,  
30 2,5-bis[ (1,3,3-trimethyl-2-indolinylidene)ethylidene]  
cyclopentanone and  
2-[ (3-ethyl-2-benzothiazolinylidene)ethylidene]cyclo-  
pentanone.  
35 7. A light sensitive photographic silver halide emulsion  
spectrally sensitized with 2,5-bis[ (3-ethyl-2-benzothiaz-  
olinylidene)ethylidene]cyclopentanone.  
40 8. A light sensitive photographic silver halide emulsion  
spectrally sensitized with 2,5-bis[ (1,3,3-trimethyl-2-indo-  
linylidene)ethylidene]cyclopentanone.

## References Cited

UNITED STATES PATENTS

- |           |         |                  |        |
|-----------|---------|------------------|--------|
| 2,860,984 | 11/1958 | Jones            | 96-140 |
| 3,140,182 | 7/1964  | Haseltine et al. | 96-141 |
| 3,148,065 | 9/1964  | Craig et al.     | 96-140 |

## FOREIGN PATENTS

- 595,785 12/1947 Great Britain.

J. TRAVIS BROWN, Primary Examiner

U.S. Cl. X.R.

96—127, 141; 260—240.1